

Patented Nov. 17, 1925.

1,562,217

# UNITED STATES PATENT OFFICE.

JOSEPH ERNEST FLEURY, OF THREE RIVERS, QUEBEC, CANADA.

## CONTROL OF BISULPHITE-PULP COOKING.

No Drawing.

Application filed May 14, 1924. Serial No. 713,344.

To all whom it may concern:

Be it known that I, JOSEPH ERNEST FLEURY, a subject of the King of Great Britain, residing at Three Rivers, in the 5 county of St. Maurice and Province of Quebec, Canada, have invented certain new and useful Improvements in the Control of Bisulphite-Pulp Cooking; and I do hereby declare that the following is a full, clear, and 10 exact description of the invention, such as will enable others skilled in the art to which it appertains to make and use the same.

This method for the control of bisulphite pulp cooking determines rapidly the quality 15 of the pulp, guarantees the uniformity of the product by giving the exact moment to blow a digester according to the desired quality of the pulp; or briefly indicates how the cooking is proceeding.

20 This method is based on the following principle:

The carbohydrates or aldehydes which have a compound action, such as sugars, 25 gums, lignins, resins, when in solution turn yellow and then brown when they are heated with an alkaline hydroxide, on account of a resinification. However, the great facility with which those alcohol groups and aldehydes are changed into carboxyls 30 by oxidation, makes it necessary to stop that reaction by alcoholation.

By testing a sample of the solution in a colorimeter, I am able to determine the bleach of the pulp, i. e., the percentage of 35 calcium, hypochlorite containing 35% active chlorine required to bleach the pulp in the digester.

The operation of the invention is as follows:

40 When a digester is working, that is, during the reaction, which begins at 105° C., I take a sample of the liquor, let it be 50 cubic centimeters, I add 25 cubic centimeters of ammonium hydroxide (one into five) 45 and 25 cubic centimeters of alcohol (ethyl or methyl) one into one. Then the liquor takes a colour more or less deep according to the quantity of carbohydrates or aldehydes with a compound action, dissolved in the 50 liquor at that moment during the cooking.

There is also precipitation of calcium and magnesium monosulphites which I eliminate by filtration.

55 The filtrate is compared in a colorimeter after having been first diluted according to the requirements of the colorimeter used.

Knowing beforehand two points on the colorimeter corresponding to two qualities of different pulps of which I have found the strength and bleach by several repeated 60 tests, I am able to determine the quality of the pulp in the digester and to compare it with the standard.

For fixing those two points on the scale of the colorimeter, I take samples of liquors from two blown digesters. I treat the liquors in the above manner and examine the filtrate in a Hess-Ives tint colorimeter. Then I determine the strength and bleach 65 of the two samples of pulp from the two digesters, using the Canadian Forest Product Laboratory methods. I find the bleach of the two pulps to be, say, 10% and 9%. I then dilute the two liquors so that they 70 read 10 and 9 respectively on the colorimeter with the green glass. The same dilution used in tests of undetermined samples 75 enables me to read the bleach, at any period of the cooking, directly from the colorimeter. In this manner, the bleach of the pulp is easily controlled and the digester may be blown when the desired bleach has been attained.

The strength of the pulp is to some extent proportional to the final bleach, depending, of course, on the condition of the digester at starting. The strength table can be compiled for a number of samples which have been tested in the colorimeter at the beginning and end of the cooking and also tested 80 for strength by a known method. A system of interpolation for other samples can then be worked out from the table.

Furthermore my method allows one to 85 judge the condition of the cooking and to determine the quality of the pulp, and the right moment to blow a digester with a product conformable to the desired standard. With the method now commonly in use, which consists in blowing a digester 90 when by titration with iodine there is a certain amount of  $SO_2$  present in the liquor, it is practically impossible to have a standard pulp for several consecutive digesters, and the quality of the product is known 95 only several hours after the digester is blown.

The new method has the advantage of 100 permitting an increased saving of steam, and this is due to the fact that the method 105 indicates when the cooking is completed and hence the steam can be shut off.

However, I know that ammonia has been used for a long time for detecting the quantity of lime present at the end of the cooking, so that a certain indication of the condition of the cooking is given; but the principle on which my method is based has never been used to determine the qualities of the pulp; and I am the first to apply the reaction of organic matters dissolved in the cooking liquor with an alkaline hydroxide, and I am also the first to prevent the formation of carboxyls by the use of alcohol.

Having thus fully described the invention, what I claim as new and desire to protect by Letters Patent is:—

1. Method of control of bisulphite pulp cooking by the colour of the liquor, consisting in drawing a sample of the liquor from a digester in operation, to which sample is added an alkaline hydroxide and an alcohol,

filtering the liquor and diluting it in determined proportion and then comparing it in a colorimeter with a predetermined graduation corresponding to certain percentages of strength and bleach of finished pulp.

2. Method of controlling bisulphite pulp cooking by the coloration of the liquor, consisting in drawing 50 c. c. of liquor from a digester in operation, adding to this liquor 25 c. c. of ammonium hydroxide (one into five) and 25 c. c. of alcohol (one to one), then filtering to remove the precipitate, diluting the filtrate to a predetermined proportion depending on the colorimeter requirements, and determining the quality of this filtrate with the aid of the colorimeter which has graduations corresponding to the strength and bleach of two different qualities of "finished pulp".

JOS. ERNEST FLEURY.